

# United States Patent Office

2,890,097

Patented June 9, 1959

1

2,890,097

## SHRINKPROOFING TEXTILES WITH POLYAMIDES AND VOLATILE POLYPOXIDES

Thompson J. Coe, Albany, Calif., assignor to the United States of America as represented by the Secretary of Agriculture

No Drawing. Application May 12, 1958  
Serial No. 734,799

4 Claims. (Cl. 8—128)

(Granted under Title 35, U.S. Code (1952), sec. 266)

A non-exclusive, irrevocable, royalty-free license in the invention herein described, throughout the world for all purposes of the United States Government, with the power to grant sublicenses for such purposes, is hereby granted to the Government of the United States of America.

This invention relates to and has among its objects the provision of novel processes for shrinkproofing and felt-proofing textiles. The invention also includes the provision of improved textiles having superior qualities as to resistance to shrinking and felting. Further objects and advantages of the invention will be evident from the following description.

It is well known in the art that many textile fibers exhibit poor dimensional stability. For example, laundering causes severe shrinkage of woolen textiles. This technical disadvantage seriously restricts the applications of wool in the textile industry and much research has been undertaken in order to modify the natural fiber in order to improve its shrinkage properties. In general, known methods of treating wool to improve its shrinkage characteristics have the disadvantage that the hand of the fabric is impaired, or, if the amount of agent applied is limited to avoid impairment of hand, the degree of shrinkage protection is relatively poor.

In accordance with the invention, wool, or other textile material, is impregnated with a polyamide then cured by subjecting to the vapors of a volatile polyepoxide. This procedure yields a product which is virtually shrink-proof under normal laundering procedures while the hand, resiliency, porosity, tensile strength, color and other valuable properties of the textile are retained. Additionally the treated textile exhibits a great improvement in resistance to creasing and wrinkling as compared to the original textile.

The prior art discloses methods for shrinkproofing textiles by applying polyepoxides and curing the polyepoxide with various curing agents, including triethylamine, ethylene diamine, diethylene triamine and other amino compounds. The process of the invention affords many advantages over the known procedure, as follows:

(a) In the process of the invention the original color of the textile is retained. For example, white wool treated in accordance with the invention retains its white color. In the known process the treated wool develops yellowness. Dyed woolen textiles treated in accordance with the invention retain their original colors in undiminished brightness whereas the processes of the prior art cause a graying or dulling of the fabrics.

(b) The process of the invention yields products of especially soft and resilient properties and more shrink-proofing effect is attained per unit weight of resinous material deposited on the fibers.

(c) The curing treatment of the invention—involving contacting the polyamide-impregnated textile with a polyepoxide in the vapor phase—has the advantage that this curing agent can penetrate readily into the textile and ensure complete and uniform cure of the polyamide com-

2

position. Moreover, the vapor phase polyepoxide treatment does not disturb the appearance, dimensions, or construction of the textile. There is no change in nap, no wrinkling. Textiles having pleats, folds, etc. retain such forms without change. Also, since the curing involves a vapor phase rather than the usual liquid treatment, no wringing or other mechanical treatments are required. This means that no wrinkling or other change in the construction or arrangement of the textile is involved.

In applying the process of the invention in practice, the textile is first impregnated with a liquid preparation containing the polyamide. The impregnation is performed in any of the usual ways. For example, the polyamide composition is applied by spraying, brushing, dipping, etc. To assist in wetting the textile, it may be run through padding rolls or the like. Excess liquid may be removed by passing the textile through wringer rolls. The proportion of active material in the liquid preparation is usually so selected that there is deposited on the textile about 0.5% to 10% of its weight of the polyamide. In general, the greater the proportion of this agent, the greater will be the shrinkage protection afforded. After the textile has been impregnated with the polyamide preparation it is cured directly or dried in air prior to curing, the latter procedure being generally preferred.

Curing of the polyamide-impregnated textile involves subjecting it to the vapors of a volatile polyepoxide. This may conveniently be done, for example, by hanging the textile in a chamber in which is exposed an open vessel containing the polyepoxide. To increase the vapor pressure of the polyepoxide, that is, the proportion thereof present in the atmosphere within the chamber, the chamber may be heated, evacuated, or both heated and evacuated. No special precautions need be taken as to addition or elimination of moisture from the system. The textile is allowed to remain in contact with the polyepoxide vapors until the polyamide is cured—that is, until it is rendered insoluble so that it is not removable from the textile by laundering. The temperature within the chamber may be at room temperature or may be increased to about 150° C. to obtain faster cure. The time for cure will vary depending on several factors such as temperature (higher temperatures promote faster cure); the nature of the polyepoxide (more volatile polyepoxides under the same conditions will cause faster cure); and the pressure within the curing chamber (generally a lower pressure will cause more polyepoxide to be vaporized, hence the cure will be faster). The curing operation is generally complete when the polyamide deposit on the textile increases in weight by about 10 to 100% due to reaction of the polyepoxide with the polyamide on the textile fibers producing an insoluble resinous composition thereon. No effort is made to control the amount of polyepoxide other than to ensure that the chamber at all times contains vaporous polyepoxide so that an excess of this reagent is always available for reaction with the polyamide.

The polyamides used in accordance with the invention are those derived from aliphatic polyamines and polybasic acids. Methods of preparing these polyamides by condensation of polyamines and polycarboxylic acids are well known in the art and need not be described here. One may prepare polyamides containing free amino groups or free carboxylic acid groups or both free amino and free carboxylic acid groups. Generally it is preferred to employ polyamides which contain free amino groups since the active hydrogens on these groups are especially reactive with the epoxy groups of the polyepoxide to form insoluble polyepoxide-polyamide reaction products. The polyamides may be derived from such polyamines as ethylene diamine, diethylene

triamine, triethylene tetramine, tetraethylene pentamine, 1,4-diamino butane, 1,3-diaminobutane, hexamethylene diamine, 3-(N-isopropylamino) propylamine, 3,3'-imino-bispropylamine, and the like. Typical polycarboxylic acids which may be condensed with the polyamines to form polyamides are glutaric acid, adipic acid, pimelic acid, suberic acid, azelaic acid, sebatic acid, isophthalic acid, terephthalic acid, beta-methyl adipic acid, 1,2-cyclohexane dicarboxylic acid, malonic acid and the like. Depending on the amine and acid constituents and the conditions of condensation, the polyamides may have molecular weights varying about from 1,000 to 10,000 and melting points about from 20-200° C. Particularly preferred for the purpose of the invention are the polyamides derived from aliphatic polyamines and polymeric fat acids. Such products are disclosed for example by Cowan et al., Patent No. 2,450,940. Typical of these polyamides are those made by condensing ethylene diamine or diethylene triamine with polymeric fat acids produced from the polymerization of drying or semi-drying oils, or the free acids, or simple aliphatic alcohol esters of such acids. The polymeric fat acids may typically be derived from such oils as soybean, linseed, tung, perilla, oiticica, cottonseeds, corn, tall, sunflower, safflower, and the like. As well known in the art, the fat acids combine to produce a mixture of dibasic and higher polymeric acids. Usually the mixture contains a preponderant proportion of dimeric acids with lesser amounts of trimeric and higher polymeric acids, and some residual monomeric acid. A typical polyamide of this type is, for example, one produced by heating soybean dimeric fatty acids and diethylene triamine.

The polyamide is preferably applied to the textile material in the form of a solution or dispersion to ensure uniform impregnation of the fibrous elements. Aqueous solutions may be used, for example, where the selected polyamide is soluble in this medium. In many cases other volatile solvents may be required such as acetone, benzene, alcohol, ethylene glycol monomethyl ether, ethylene glycol monoethyl ether, dioxane, etc. depending on the property of the agent in question. It is often preferred to apply the polyamide in the form of aqueous emulsions prepared by application of any of the known emulsification technique. A preferred procedure is to dissolve the polyamide in a suitable quantity of alcohol or other volatile organic solvent and add this solution to water with vigorous agitation. In this way contact of the solution with water will precipitate the polyamide in minute particles which will be relatively easy to emulsify. To assist in forming and maintaining the emulsion one may add a small proportion of a conventional emulsification agent. For this purpose one may employ agents such as soaps, long-chain alkyl sulphates, long-chain alkyl benzene sulphonates, alkyl esters of sulphosuccinic acid, etc., typical examples being sodium lauryl sulphate, sodium alkyl ( $C_{10}-C_{20}$ ) benzene sulphonate, sodium dioctylsulphosuccinate, etc. Preferably, emulsifying agents of the non-ionic type are employed, for example, sorbitan laurate, polyoxyethylene ether of sorbitan laurate, polyoxyethylene ether of sorbitan monostearate, polyoxyethylene ether of sorbitan distearate, sorbitan trioleate, iso-octyl phenyl ether of polyethylene glycol, and so forth. Other suspending agents as gums, gelatin, pectin, soluble starch, dextrins, etc. can be used to keep the polyamide in suspension. It is obvious that the proportion of active materials in the solution or dispersion may be varied as necessary to deposit on the textile material the desired percentage of polyamide.

Butadiene dioxide (also designated 1,2,3,4-diepoxybutane) is preferred as the polyepoxide for use in the process of the invention. However other volatile polyepoxides may be employed as for example 1,2,5,6-di-epoxyhexane, 1,2,4,5-diepoxyhexane, isoprene dioxide,

limonene dioxide. Volatile polyepoxide ethers may also be employed as for example diglycidyl ether, diglycidyl thioether, diglycidyl ether of ethylene glycol, and the like. In general, one may employ any volatile polyepoxide which contains at least two epoxy



groups and wherein the remainder of the polyepoxide molecule is a carbon chain or a carbon chain interrupted with ether linkages. Preferably the polyepoxides are free from functional groups other than hydroxyl groups, ether groups, and epoxy groups.

The process of the invention is particularly adapted to the treatment of wool but is also advantageously applicable to other textiles including mohair; animal hair; silk; fibers made from proteins such as zein, casein, peanut protein, soybean protein, keratins, etc.; cotton; regenerated cellulose; viscose; linen; cellulose acetate; etc. The textile material may be in the form of fibers, threads, yarns, woven or knitted fabrics, garments, etc.

The invention is further demonstrated by the following illustrative examples.

#### Example I

Pieces of white woolen cloth were padded with emulsions of a polyamide. In these emulsions, the total concentration of this agent was varied (as set forth below): In each case 2% of the iso-octylphenyl ether of polyethylene glycol (Triton X-100) was used as the emulsifying agent. The polyamide was a commercial product being a condensation product of diethylene triamine and heat-dimerized unsaturated fat acids. It was a viscous liquid at ordinary temperatures with a viscosity of  $A_3-A_1$  on the Gardner-Holt scale at 25° C. and a specific gravity of 0.99 at 25° C.

The impregnated cloth samples were dried in air at 65° C. then placed in a chamber which contained an open vessel of butadiene dioxide. The samples were exposed to the polyepoxide vapors for 72 hours at room temperature. It was observed that all the cured samples were white in color.

The treated samples of cloth and a sample of untreated cloth (control) were subjected to tests to determine their shrinkage characteristics. In these tests the cloth samples were subjected to a laundering operation wherein the cloth was violently agitated in an "Accelerator" for 3 min. in a 0.5% solution of sodium oleate at 40° C. with a cloth to solution ratio of 1 to 35. The area of the cloth was measured before and after laundering. The washing tests were carried out in duplicate. The results are tabulated below, the shrinkage values being averages of the duplicate tests.

| Sample       | Cone. of polyamide in emulsion, percent | Pickup of polyamide by cloth, percent | Pickup of cured polyamide polyepoxide by cloth, percent | Area shrinkage after laundering, percent |
|--------------|-----------------------------------------|---------------------------------------|---------------------------------------------------------|------------------------------------------|
| a.....       | 5                                       | 3.7                                   | 5.1                                                     | 0                                        |
| b.....       | 3                                       | 2.8                                   | 3.95                                                    | 0                                        |
| c.....       | 1                                       | 2.1                                   | 3.3                                                     | 19                                       |
| control..... |                                         |                                       |                                                         | 54                                       |

Having thus described the invention, what is claimed is:

1. The method of shrinkproofing a textile without significant impairment of its hand which comprises impregnating the textile with a polyamide of an aliphatic polyamine and a polycarboxylic acid, said polyamide containing free groups selected from the group consisting of amine groups and carboxyl groups, the total amount of polyamide deposited on the textile being about from 0.5 to 10% of the weight of the textile, and exposing the impregnated textile to a volatile polyepoxide in the

vapor phase to cure and insolubilize the polyamide on the textile fibers, the polyepoxide containing at least two epoxy



groups per molecule, the remainder of the polyepoxide molecule being a member selected from the group consisting of a carbon chain and a carbon chain interrupted with ether linkages.

2. The method of claim 1 wherein the polyepoxide is butadiene dioxide.

3. The method of shrinkproofing wool without significant impairment of its hand which comprises impregnating wool with a polyamide of an aliphatic poly-amine and a polymeric fat acid containing at least two carboxyl groups, said polyamide having free amine

groups, the total amount of polyamide deposited on the wool being about from 0.5 to 10% of the weight of the wool and exposing the impregnated wool to a volatile polyepoxide in the vapor phase to cure and insolubilize the polyamide on the wool fibers, the polyepoxide containing at least two epoxy



10 groups per molecule the remainder of the polyepoxide molecule being a member selected from the group consisting of a carbon chain and a carbon chain interrupted with ether linkages.

4. The method of claim 3 wherein the polyepoxide is butadiene dioxide.

No references cited.